

Patented Oct. 7, 1924.

1,510,983

# UNITED STATES PATENT OFFICE.

SAMUEL H. DOLBEAR, OF SAN FRANCISCO, CALIFORNIA, ASSIGNOR OF ONE-HALF TO EDWIN LETTS OLIVER, OF SAN FRANCISCO, CALIFORNIA.

## METHOD OF CONCENTRATING OIL SHALES.

No Drawing.

Application filed November 11, 1920. Serial No. 423,317.

To all whom it may concern:

Be it known that I, SAMUEL H. DOLBEAR, a citizen of the United States, residing at San Francisco, in the county of San Francisco and State of California, have invented new and useful Improvements in Methods of Concentrating Oil Shales, of which the following is a specification.

This invention relates to a method of 10 treating oil shales and has for its object to separate the valuable organic compounds in the shale from the waste or gangue which produces no oil.

Usually the oil does not exist as such 15 in the shale and when present is found in very minute quantities, but is produced by the destructive distillation of complex organic compounds in the shale. Destructive distillation, that is, heating in the 20 absence of air, decomposes this organic matter and yields hydrocarbon oils and permanent gases.

In carrying out my object I concentrate 25 the valuable organic compounds present in the oil shale by subjecting a pulp of oil shale to flotation.

In flotation as heretofore practiced, advantage is taken of the selective preference 30 of oil for the metallic and certain metalloid particles such as graphite, present in the ore. I have discovered that oil and some other substances have a selective affinity 35 for certain organic substances present in oil shales and that if the shales are finely ground and mixed with water and a suitable quantity of oil or other selective reagents be present, and the mixture aerated, bubbles will be formed to which the valuable organic compounds attach themselves and are brought to the surface by the bubbles and are retained in the froth formed at the surface. The froth may then be readily separated from the liquid. All organic substances do not exhibit this characteristic 45 of selective preference to oil, and it is believed that the cohesion of the two in the present invention is due to the natural preference of certain oily liquids for related hydrocarbon solids.

At present there are no shale oil operations 50 in this country that have reached commercial production, although there is a great deal of activity, particularly in the States of Colorado, Utah and Montana where there are large and easily accessible deposits of

rich shale. The chief reason for the failure to produce oil commercially from shale in this country has been the expense in connection with destructively distilling the shale. There is present in the shale a large 60 quantity of waste or gangue which yields no oil. By separating this waste or gangue before the destructive distilling operation is carried out a great saving is effected in time, labor and fuel. 65

My invention may be practiced with many different kinds of apparatus and any of the well known machines used in the flotation of metalliferous ores may be used as desired. The steps contemplated are: grinding 70 of the shale into a pulverulent state; mixing this powdered material with water; adding a small quantity of oil to the water in cases where there is an insufficient quantity of free oil in the shale to effect a flotation, and aerating the pulp or mixture by introducing air through it to create a froth, which froth will rise to the surface carrying with it the valuable organic compounds present 75 in the shale while the earthy substances present, such as silicious material, gypsum and other inorganic compounds sink. Thereafter the valuable portion may be skimmed off and destructively distilled in the usual way to extract the oil and other valuable 80 ingredients therefrom. 85

In practicing this process it is necessary to have present a small quantity of oil or other flotative reagent in the pulp, the character and quantity of which must be determined by preliminary tests. If, however, the shales are found to contain free oil in such quantity as to act as a flotative agent then no oil need be added. In using the term "oil shales" herein I do not refer 90 to shales in which a substantial amount of free oil is present, such for instance as some of the shales found in California. 95

In the concentration of some shales it may be desirable to add an electrolyte, such as 100 sulfuric acid, especially where the earthy material has a tendency to slime or become colloidal on grinding. The amount and character of such electrolyte must be determined by preliminary tests. 105

Having thus described my invention, what I claim and desire to secure by Letters Patent is:—

1. A method of recovering oil from shale which consists of converting such 110

shale into a liquid pulp, subjecting the pulp to froth flotation, separating the resultant froth from the remainder and destructively distilling only those particles taken off with the froth.

2. A method of recovering oil from shale which consists in reducing the shale to a pulverulent state, mixing the same with water, aerating the mixture so formed to 10 produce a froth on the surface, separating the froth from the remainder and destructively distilling only those particles taken off with the froth.

3. A method of recovering oil from shale 15 which consists in reducing the shale to a pulverulent state, forming a pulp thereof

by the addition of water and a small quantity of flotation reagent, aerating the pulp so as to produce a froth on the surface and separating the resultant froth from the remainder and destructively distilling only those particles taken off with the froth.

4. A method of recovering oil from shale which consists in reducing the shale to a pulverulent state, forming a pulp thereof 25 by the addition of water and an electrolyte, aerating the pulp so as to produce a froth on the surface, separating the resultant froth from the remainder and destructively distilling only those particles taken off with the froth.

SAMUEL H. DOLBEAR.